

# United States Patent Office

3,220,847

Patented Nov. 30, 1965

1

3,220,847

## PHOTOGRAPHIC GELATIN LAYERS CONTAINING THE WATER-SOLUBLE SALTS OF VARIOUS HALF ESTERS OF SUBSTITUTED SUCCINIC ACID AS COATING AIDS

William J. Knox, Jr., Rochester, N.Y., and Robert E. Sticker, Lawrence, Kans., assignors to Eastman Kodak Company, Rochester, N.Y., a corporation of New Jersey  
No Drawing. Filed Feb. 23, 1962, Ser. No. 175,284  
13 Claims. (Cl. 96—94)

This invention relates to coating aids for gelatin coating solutions particularly those used for photographic purposes which are in the nature of water-soluble salts of half esters of branched-chain substituted succinic acids.

In the application of gelatin coating compositions, particularly gelatin-silver halide photographic emulsions, to a support such as film base or paper, it is desirable that there be present therein a coating aid to facilitate the application of the gelatin layer to the surface of the support. This application of gelatin compositions can be either in the form of a single layer or in multilayer form such as by the simultaneous application of a plurality of layers to a support. The presence of coating aids in the coating or coatings assists in obtaining layers which in the form of dry coatings are free of defects such as repellencies, pencil line streaks, and the like. In such coating operations, however, the coating aids that induce adequate rewettability of the gelatin layer usually also impart slickness or slipperiness thereto. This surface slickness in photographic products is generally objectionable because of difficulties in handling and the possibility of telescoping when film is in roll form. It has often been necessary to use a mixture of two different surfactants to impart both surface roughness and rewettability to gelatin coatings. The mixing of two different coating aids is often times undesirable, and some of the materials which have been proposed for that pur-

2



one of  $\text{R}_1$  and  $\text{R}_2$  being H, the other being selected from the group consisting of alkyl and alkenyl radicals containing 8-16 carbon atoms having at least two points of branching; M is a cation such as Na, K,  $\text{NH}_4$  or alkylammonium; Q is the radical derived from a water-soluble alcohol containing 3-19 oxygen atoms in the form of hydroxyl or ether groups; and  $n$  is an integer from 1-8, being 1 when Q is the radical derived from a monohydroxy alcohol and 2-8 when Q is the radical derived from a polyhydroxy alcohol.

It may be seen that generally two isomeric forms of the compounds of our invention are possible. Thus, referring to the generic formula shown above, it is apparent that the branched-chain alkyl or alkenyl radical may be positioned on the succinic radical beta or gamma to the half ester. It is believed (but not known) that one isomer predominates in the normal preparation of the compounds of this invention. In any event, a mixture of the isomers appears satisfactory in employing the compounds of the invention as coating aids in protein coating compositions.

The alcohol, from which the desired half esters are derived, is not critical so long as the alcohol is a water-soluble compound containing from 3-19 oxygen atoms in the form of hydroxyl or ether groups. By the term ether we mean to include acetals and ketals also. Representative alcohols include 2-(2-ethoxyethoxy)ethanol, anhydroenneaheptitol, glycerol, sorbitol, 2,2,6,6 - tetramethylolcyclohexanol, pentaerythritol, 2,2,6,6,10,10-hexamethylol-4,8-oxaundecamethyleneglycol (trimer of pentaerythritol), and the like. A particularly useful alcohol for our purpose is a sucrose derivative, called Hyprose SP-80 hereinafter, having the formula:



pose are naturally occurring and often vary in quality or contain impurities undesirable in photographic use.

One object of our invention is to provide gelatin coating compositions from which layers having both adequate rewettability after drying and sufficient roughness of surface to facilitate handling may be obtained. Another object of our invention is to provide gelatin coating compositions from which may be prepared coatings that when dry have few if any repellencies, pencil line streaks, or other undesirable characteristics. A further object of our invention is to provide gelatin coating aids comprising certain half esters of branched-chain substituted succinic acids. Other objects of our invention will appear herein.

We have found that the water-soluble salts of various half esters of branched-chain succinic acids when incorporated in photographic emulsions or other gelatin coating compositions may be used in preparing products exhibiting good handling characteristics. Coating aids which we have found to be particularly useful when incorporated in gelatin compositions are those having the formula:

50 The compounds useful in this invention may be prepared by reacting the desired branched-chain alkyl or alkenyl succinic anhydride with the desired alcohol, followed by neutralization with a base such as sodium hydroxide. Particularly valuable coating aids may be prepared by reacting commercially available dodeceny succinic anhydride (wherein the dodecetyl radical is a mixture of branched monoolefins formed by tetramerizing propene) with an alcohol. The structural formulas of the coating aids thus produced are indicated below; it being understood that the dodecetyl substituent may be attached to either of the carbon atoms of the hydrocarbon portion of the succinic acid radical:

### COMPOUND I



### COMPOUND II



## 3

## COMPOUND III



## COMPOUND IV



## COMPOUND V



## COMPOUND VI



## COMPOUND VII



## COMPOUND VIII



## COMPOUND IX



## COMPOUND X



## COMPOUND XI



## COMPOUND XII



## COMPOUND XIII



The dodecetyl radical of the above compounds contains not less than two points of branching, and generally is a highly branched monoolefin radical. As indicated above, various other alkyl and alkenyl substituted hydrogen succinates may be employed in accordance with this invention. Representative half esters include those derived from the following acid: a hydrogen tetramethylbutylsuccinic acid, sodium salt; a hydrogen branched-chain dodecylsuccinic acid, sodium salt; a hydrogen branched-chain tridecylsuccinic acid, sodium salt; a hydrogen branched-chain pentadecylsuccinic acid, sodium salt; a hydrogen branched-chain hexadecylsuccinic acid, sodium salt; a hydrogen branched-chain nonenylsuccinic acid, sodium salt; a hydrogen branched-chain pentadecenylsuccinic acid, sodium salt; and, a hydrogen branched-chain hexadecenylsuccinic acid, sodium salt. In each of the foregoing compounds, the alkyl or alkenyl radical contains not less than two points of branching. Of course the half ester portion in these compounds conform to the general description of the alcohols given above.

We have found that when these compounds are in-

## 4

corporated in small amounts in aqueous solutions of gelatin good coating properties are obtained. This has been found to be true both in coating operations in which a single layer has been applied to film base or paper in mixed coating operations such as described in U.S. 2,761,991 of T. A. Russell. It was found that any amount of coating aid present in the gelatin composition was effective, however, it is convenient to operate within the coating range of 0.5-15%, based on the weight of the gelatin, and preferably 1-10% is employed.

In the coating aids in accordance with our invention it is desirable that the branched-chain substituent attached to the hydrocarbon portion of the succinic acid radical have 8-16 carbon atoms. In many cases as will be noted from the formulae, the radical derived from an alcohol will be that derived from a polyhydroxy alcohol and therefore the compounds can comprise more than one succinyl group per unit structure of compound.

The following examples illustrate the preparation of compounds useful as coating aids in accordance with our invention.

## Example A

A homogeneous mixture of 532 parts (2.0 moles) of dodecenylsuccinic anhydride and 268.4 parts (2.0 moles) of 2-(2-ethoxyethoxy)ethanol was heated on a steam bath for four hours. The resulting product was cooled to room temperature, diluted with 1000 parts of water and while stirring was neutralized with 80 parts (2.0 moles) of sodium hydroxide in 10% aqueous solution. After mixing for one hour, the solution was diluted with water to represent a 25% solution of coating aid, i.e. 2-(2-ethoxyethoxy)ethyl hydrogen dodecenylsuccinate, sodium salt (Compound I).

## Example B

A mixture of 56.6 parts (0.213 mole) of dodecenylsuccinic anhydride, 38.8 parts (0.213 mole) of sorbitol and 0.5 part of anhydrous p-toluenesulfonic acid were mixed into 200 parts of acetone and the mixture was refluxed for four hours. Acetone was then boiled off from the resulting clear solution to give a clear, yellow liquid which was diluted with 100 parts of water and neutralized with 8.5 parts (0.213 mole) of sodium hydroxide, in 10% aqueous solution.

The mixture while stirring was heated on a steam bath for two hours and then was diluted with water to form a 20% solution of coating aid, i.e. sorbityl hydrogen dodecenylsuccinate, sodium salt (Compound IV).

## Example C

32.1 part (0.236 mole) of pentaerythritol and 62.8 parts (0.236 mole) of dodecenylsuccinic anhydride were mixed and the mixture was heated for fifteen minutes at 195-210° C. The mixture was allowed to cool to 80° and was then diluted with 100 parts of water. While stirring and maintaining the temperature at 70° C., there was added 9.4 parts (0.236 mole) of sodium hydroxide in 10% aqueous solution. The mass was mixed for an hour and was diluted to form a 25% solution of coating aid, i.e. pentaerythritol hydrogen dodecenylsuccinate, sodium salt (Compound XI).

Pentaerythritol tris(hydrogen dodecenylsuccinate, sodium salt) (Compound XII) was prepared in a similar manner but proportionate amounts of materials were employed.

## Example D

The water was removed from 59.5 parts (0.196 mole) of 70% aqueous anhydroenneahexitol by evaporation, in vacuo, on a steam bath. Thereupon 52.2 parts (0.196 mole) of dodecenylsuccinic anhydride were added and the stirred mixture was heated for 30 minutes at 160-170° C. Cooling to room temperature resulted in a yellow, tacky, clear glass which was powdered and dissolved in 7.8 parts (0.196 mole) of sodium hydroxide in 10% aqueous solution. The resulting solution was diluted

with water to form a 25% solution of the coating aid, i.e. the sodium salt of 3,3,5,5-tetramethylol-4-byranol monoester of dodecenylsuccinic acid (Compound II). The disodium salt of the diester of 3,3,5,5-tetramethylol-4-byranol was prepared in a similar manner from 2 moles of dodecenylsuccinic anhydride per mole of anhydroen-neaheptitol.

*Example E*

A mixture of 73.7 parts (0.0913 mole) of Hyprose SP-80 [octakis(2-hydroxypropyl)sucrose] and 24.3 parts (0.0913 mole) of dodecenylsuccinic anhydride was heated at 140-160° C. A homogeneous mixture was obtained and was allowed to cool to 80° C. and was then diluted with 100 parts of water and neutralized with 3.7 parts of sodium hydroxide while maintaining the temperature at 60-70° C. After a thorough mixing, the solution was diluted to form a 20% solution of coating aid (Compound VII).

In a similar manner Hyprose SP-80 tris(hydrogen dodecenylsuccinate, sodium salt) (Compound VIII), Hyprose SP-80 pentakis(hydrogen dodecenylsuccinate, sodium salt) (Compound IX), and Hyprose SP-80 heptakis(hydrogen dodecenylsuccinate, sodium salt) (Compound X), were prepared using proportional amounts of materials in their preparation.

The following examples illustrate the use of these coating aids in applying coatings. A coating experiment in which an aqueous solution of gelatin was applied by a hopper coating method as a single layer to cellulose ester film base using 0.22 gram of the coating aids designated per pound of coating composition.

The following results were obtained:

| Coating Aid          | Repel-lencies<br>(25 ft. <sup>2</sup> ) | Mottle       | Longi-tudinal<br>Streaks |
|----------------------|-----------------------------------------|--------------|--------------------------|
| Control (none) ----- | 10                                      | Sl. -----    | Sl. -----                |
| Compound I -----     | 0                                       | Sl. -----    | V. sl. -----             |
| Compound II -----    | 0                                       | Sl. to sl. + | Sl. -----                |
| Compound III -----   | 0                                       | V. sl. ----- | V. sl. -----             |
| Compound V -----     | 0                                       | V. sl. ----- | V. sl. -----             |
| Compound VII -----   | 0                                       | V. sl. +     | V. sl. -----             |
| Compound VIII -----  | 2                                       | V. sl. ----- | V. sl. -----             |
| Compound IX -----    | 1                                       | V. sl. ----- | V. sl. -----             |
| Compound X -----     | 0                                       | V. sl. ----- | V. sl. -----             |
| Compound XI -----    | 0                                       | V. sl. ----- | V. sl. -----             |
| Compound XII -----   | 2                                       | Sl. -----    | V. sl. -----             |
| Compound XIII -----  | 1                                       | Sl. -----    | Sl. -----                |

*Example 2*

There was simultaneously applied to paper a photographic emulsion coating and a gelatin overcoating both of which contained Compound VII by means of the coating technique described in U.S. 2,761,991 in the proportions indicated together with a control in which saponin coating aid was employed. It was found that the paper thus obtained was more responsive to developer spread than the control coatings while the coefficient of friction was not appreciably altered.

|                    | Surfactant<br>Concentration<br>emul. overcoat |          | Developer<br>Spread | Coef. of<br>Friction | Repel-lencies<br>(7.5 ft. <sup>2</sup> ) |
|--------------------|-----------------------------------------------|----------|---------------------|----------------------|------------------------------------------|
|                    | (G./lb.)                                      | (G./lb.) |                     |                      |                                          |
| Compound VII ----- | 0.13                                          | 0.5      | 12.80               | 0.398                | None                                     |
|                    | 0.25                                          | 0.5      | 10.20               | 0.320                | None                                     |
|                    | 0.5                                           | 0.5      | 11.30               | 0.332                | 2-3                                      |
| Control -----      | 0.25                                          | 0.5      | 7.55                | 0.332                | None                                     |

In the above data repellencies refers to the number of dull and uncoated spots in the area designated whether 25 square feet or 7.5 square feet.

Developer spread was determined by delivering in a standard manner one cc. of developer solution to a surface of photographically sensitized paper carrying a clear gelatin overcoat, and measuring the area which develops in a period of 30 seconds. This test indicates how effec-

tively an emulsion will wet. A developer spread of 4.0 cm.<sup>2</sup> or more is desirable.

The coefficient of friction was determined by placing the coated side of photographically sensitized paper carrying a gelatin overcoat against the uncoated side of a similar sheet. The coefficient of friction was measured to obtain the slickness of the gelatin coatings. Difficulties occur in stacking coated sheets when the coefficient of friction is less than about 0.25.

We claim:

1. A composition comprising gelatin having therein a water-soluble coating aid having the formula:



in which one of R<sub>1</sub> and R<sub>2</sub> is H, the other being selected

from the group consisting of alkyl and alkenyl radicals of 8-16 carbon atoms having at least two points of branching; M is a water solubility imparting cation; Q is the radical of a water-soluble alcohol containing 3-19 carbon atoms in the form of groups selected from the hydroxyl and ether groups and n is an integer of 1-8, being 1 when Q is a radical of a monohydroxy alcohol and 2-8 when Q is a radical of a polyhydroxy alcohol.

2. A photographic emulsion comprising silver halide grains carried by a gelatin vehicle which gelatin contains a water-soluble coating aid having the formula:



in which one of R<sub>1</sub> and R<sub>2</sub> is H, the other being selected from the group consisting of alkyl and alkenyl radicals 8-16 carbon atoms having at least two points of branching; M is a water solubility imparting cation; Q is the radical of a water-soluble alcohol containing 3-19 carbon atoms in the form of groups selected from the hydroxyl and ether groups and n is an integer of 1-8, being 1 when Q is a radical of a monohydroxy alcohol and 2-8 when Q is a radical of a polyhydroxy alcohol.

3. A composition of matter comprising gelatin containing as a coating aid therein a water-soluble salt of 2-(2-ethoxyethoxy)ethyl hydrogen dodecenylsuccinic acid.

4. A gelatin-silver halide photographic emulsion containing a water-soluble salt of 2-(2-ethoxyethoxy)ethyl hydrogen dodecenylsuccinic acid.

5. A composition of matter comprising gelatin containing as a coating aid therein a water-soluble salt of sorbityl hydrogen dodecenylsuccinic acid.

6. A gelatin-silver halide photographic emulsion containing a water-soluble salt of sorbityl hydrogen dodecenylsuccinic acid.

7. A composition of matter comprising gelatin containing as a coating aid therein a water-soluble salt of pentaerythritol hydrogen dodecenylsuccinic acid.

8. A gelatin-silver halide photographic emulsion containing a water-soluble salt of pentaerythritol hydrogen dodecenylsuccinic acid.

9. A composition of matter comprising gelatin containing as a coating aid therein a water-soluble salt of 3,3,5,5-tetramethylol-4-byranol monoester of dodecenylsuccinic acid.

10. A gelatin-silver halide photographic emulsion containing a water-soluble salt of 3,3,5,5-tetramethylol-4-byranol monoester of dodecenylsuccinic acid.

11. A composition of matter comprising gelatin containing as a coating aid therein a water-soluble salt of Hyprose-80 octakis(hydrogen dodecenylsuccinic acid).

12. A gelatin-silver halide photographic emulsion containing a water-soluble salt of Hyprose-80 octakis(hydrogen dodecenylsuccinic acid).

13. A composition of matter comprising gelatin containing the sodium salt of 2-(2-ethoxyethoxy)ethyl hydrogen dodecenylsuccinic acid as the coating aid therein.

References Cited by the Examiner

5

UNITED STATES PATENTS

|           |        |                    |         |
|-----------|--------|--------------------|---------|
| 2,240,476 | 4/1941 | Simmons et al.     | 96—109  |
| 2,899,327 | 8/1959 | Christopher et al. | 106—125 |
| 2,933,406 | 4/1960 | Salzberg et al.    | 106—125 |
| 2,937,088 | 5/1960 | Gray et al.        | 96—94   |
| 2,940,854 | 7/1960 | Gray               | 96—94   |

|           |         |               |       |
|-----------|---------|---------------|-------|
| 2,960,404 | 11/1960 | Milton et al. | 96—94 |
| 3,018,178 | 1/1962  | Harriman      | 96—94 |
| 3,026,202 | 3/1962  | Knox et al.   | 96—94 |
| 3,033,680 | 5/1962  | Milton et al. | 96—94 |
| 3,038,804 | 6/1962  | Knox et al.   | 96—94 |
| 3,042,524 | 7/1962  | Albus et al.  | 96—94 |
| 3,068,101 | 12/1962 | Knox et al.   | 96—94 |

FOREIGN PATENTS

|         |        |         |
|---------|--------|---------|
| 128,286 | 7/1959 | Russia. |
|---------|--------|---------|

NORMAN G. TORCHIN, *Primary Examiner.*